

## UNITED STATES PATENT OFFICE

2,027,271

## PRODUCTION OF NEGATIVES WITH PHOTOGRAPHIC IMAGES THEREON OF ENHANCED QUALITY

Arthur Ernest Field, London, England

No Drawing. Application June 17, 1935, Serial No. 27,125. In Great Britain December 7, 1933

2 Claims. (Cl. 95—88).

This invention relates to the production, from dry plates, paper, film or the like coated with photographic emulsions of the kind comprising silver light-sensitized materials, of negatives with photographic images thereon of considerably enhanced quality compared with that of the photographic images as originally formed on the negative by the usual methods of development applied.

10 Heretofore improvements in the quality of the photographic image on a negative by retouching, fine etching or reducing operations applied directly to the negative as such have involved considerable difficulties and frequently not enabled the desired result to be obtained owing to the fact that alterations or corrections in tone value are not clearly visible on the negative and can only be properly observed when a positive is printed from the negative.

20 Further for use in the production of photo-mechanical printing surfaces it has been usual first to prepare a diapositive from a continuous tone negative of the picture to be reproduced, to retouch or etch the diapositive so as to obtain 25 a positive having the correct colour and tone values and then to produce from the retouched or corrected diapositive a contact negative from which latter flat printing forms were produced. This method however has the disadvantage that 30 three separate plates are involved therein.

The present invention has for its object to enable negatives with photographic images thereon of greatly improved quality to be obtained by operations carried out on one and the same plate, 35 film or the like in which the retouching, fine etching or alteration of tone values is effected on an intermediately formed photographic image of positive appearance, thus overcoming various disadvantages, such for instance as those above mentioned, met with in previous methods that 40 have been proposed for the improvement of the quality of photographic images on negatives. For this purpose according to the present invention a process of treating a negative to give a 45 photographic image thereon having improved tone-printing values consists in subjecting the negative to the action of a solution of a bleaching reagent so as to produce on the plate, film or the like a photographic image of positive appearance, then effecting the required retouching, 50 etching or reducing by means of a solvent solution for the silver halide salts in the emulsion, and finally subjecting the plate, film or the like to the action of a solution which blackens the 55 silver salts image and re-converts the image of

positive appearance to a negative image. The retouched or tone-corrected negative so obtained may be used as such for printing from, or, especially in the case when the negatives are to be employed for photo-mechanical work, their density may be improved by subjecting them to an intensifying treatment with one of the usual known intensifiers with or without a re-developer. If desired the intensified negatives can be bleached again to a positive appearance, re- 10 etched or etched as may be required, re-converted to a negative and then again intensified, the whole process being repeated as desired in accordance with the final result that it is desired to obtain and the purpose for which the final negative is intended. 15

The most suitable bleaching agent for converting the original negative into one of a positive appearance is a solution of iodine in an aqueous solution of potassium iodide but there 20 may also be used one of the other well-known photographic bleachers, such as a solution of potassium ferricyanide and potassium bromide or an acid solution of potassium permanganate, such as a solution of potassium permanganate acidified with acetic or hydrochloric acid. 25

It is to be understood that throughout the present specification and claims the expression "bleaching reagent" is intended to comprise solely those chemical reagents which convert the 30 silver image on a fixed plate to a silver halide image of positive appearance and that the term does not include mercury salts which are used to form a bleached silver-mercury-chloride image as a preliminary step in the ordinary intensification processes. 35

For effecting the re-touching or etching on the plate or film of positive appearance obtained as above mentioned there may conveniently be employed an aqueous solution of potassium cyanide, 40 any parts of the positive image which it is desired to protect from the action of the potassium cyanide or other solvent for the silver halide salts being coated with an appropriate reducer-resisting agent such as a varnish, as for example a 45 cellulose varnish, or litho crayon.

The following is a description of one method of carrying the present invention into effect:—

An exposed photographic dry plate is developed in the usual manner, for example with known developing solutions such as hydroquinone—caustic or metol quinol, rinsed in water and fixed so as to produce a negative which, on subjection to the etching or reduction operation, will leave a clean 50 55

image. A suitable fixing bath is for example one of the following known composition:—

|                              |          |
|------------------------------|----------|
| Sodium thiosulphate crystals | 2½ lbs.  |
| Sodium bisulphite            | 4 ozs.   |
| 5 Potassium iodide           | ¾ oz.    |
| Water to make                | 1 gallon |

After the plate has been fixed and washed it is converted to one of a positive appearance by 10 bleaching it with a solution of iodine in potassium iodide, for example a solution containing 88 grains iodine, 3 oz. potassium iodide and 60 oz. water. The plate is then washed with water until it is of clear positive appearance, the washing 15 operation being hastened if desired by first removing excess of iodine solution from the plate by immersing it in an aqueous solution of potassium hydroxide such as a solution of 1 oz. caustic potash (sticks) in 80 oz. water. In the case 20 where the bleaching of the negative is effected with a solution of potassium permanganate acidified with acetic or hydrochloric acid, the plate is well washed with water and then immersed in an aqueous solution containing about 5 per cent of 25 potassium meta-bisulphite so as to remove permanganate stains. When the bleached plate has been well washed with the potassium hydroxide or meta-bisulphite solution, as the case may be, so as to be quite clear from iodine streaks or 30 permanganate stains, it is rinsed in water and dipped for a short time, for instance about 10 seconds at ordinary atmospheric temperature, in a silver halide solvent solution such as an aqueous solution of hypo (sodium thiosulphate), potassium iodide, potassium cyanide or other known 35 reducers. After treatment in the dipping bath as just mentioned, whereby a clear image free from stains is ensured, the reduction or etching effect of the dipping bath is stopped by the action 40 of water, the plate being rinsed well in water after which it may be dried or left damp as desired for the next step. If all parts of the image now have the required tone then the next step 45 is to re-convert the positive to a negative image in the manner described in detail hereafter by treating the plate with a solution which blackens the silver salts image. On the other hand if, as is more frequently the case, a further reducing 50 or etching action of certain parts of the image is required to produce alterations of tone, varnish or litho crayon or other reducer-resisting agent is applied to those parts of the image which already have the required tone and that 55 it is desired to protect from the action of the reducing bath, comprising a solvent solution for the silver halide salts, to which the plate is next subjected. After the plate has been treated where necessary by varnish or other reducer 60 resisting agent it is washed and dipped for a short time, for example ten seconds, in an aqueous solution of potassium cyanide (for example a solution consisting of 5 parts of a ten-per-cent stock solution of potassium cyanide and 145 parts water) whereby the varnished parts of the image 65 will now stand out more prominently from the unvarnished portions which latter become heavier in tone as a result of the action of the reducing bath. The plate is then immediately washed in water to stop the reducing action of the potassium cyanide solution on the unvarnished portions of the plate. Plates may be varnished and 70 reduced as many times as required in order to obtain the desired effect, and differences in tonal 75 values may be corrected or emphasized as re-

quired in accordance with the strength of the reducing bath and the time during which the plate is immersed therein. The use of litho crayon instead of varnish as the reducer resisting agent gives an edge which is softer than that obtained by varnish. After the re-touching or etching of the plate has been completed the varnish or other reducer-resisting agent is removed by the aid of a suitable solvent, whereupon the plate is treated with a dilute acid solution, for example a dilute 10 solution of nitric (e. g. commercial nitric acid 3 parts, water 60 parts) or acetic acid, for a short time, say about 20 seconds, in order to remove from the plate the silver residue which is left as a scum. The plate is then washed with water 15 and the image thereon re-converted into a negative image by blackening the silver salts image in a suitable solution such as an aqueous solution containing about 0.5 per cent sodium sulphide or a solution containing a developer such as 20 for instance as metol hydroquinone (thorough blackening being assisted if need be by exposure to light), or a solution containing both sodium sulphide and a developer. After the negative image has thus been re-formed on the plate it is 25 again washed and, after drying, may, for certain kinds of work, be printed from without further treatment. Where the negative is to be used for photo-mechanical work and the like its density may be improved by treatment with known intensifying agents such as mercuric chloride, bromide or iodide, or the contrast or stencil effect 30 may be strengthened by the use of a redeveloper-intensifier mixture such as one comprising adurol 1½ parts, citric acid 1 part, water 80 parts mixed 35 with a five-per-cent solution of silver nitrate (slightly acidified with nitric acid) in the proportion of about three parts of the adurol solution to one part of the silver nitrate solution. In place of the adurol solution there may be employed 40 solutions of other plate-developing chemicals such as hydroquinone or metol. When the negative under treatment is a half-tone plate the half-tone dots, which have been reduced in size by treatment with the reducer (i. e. the silver 45 halide solvent) are not restored to their original size by the subsequent treatment with the redeveloper-intensifier mixture although their density is increased, since in the present process the dot opacity increases more than dot size during the 50 aforesaid treatment with the redeveloper-intensifier. This enables the half-tone dots to be greatly reduced in size and yet brought to a substantially uniform density of the required degree, a result which has not been possible in the 55 processes heretofore employed where on re-development the dot opacity does not increase more than dot size. Thus by means of the method according to the present invention negatives can 60 be produced showing increased contrast and density with little alteration to image size.

The negatives after intensification are then ready for use in photo-mechanical printing work.

If found necessary or desirable the plates after 65 having been subjected to re-development with the adurol and silver nitrate solution can be bleached again in an iodine solution, retouched or reduced where necessary, and then re-converted to a negative by blackening in the manner 70 previously described.

By means of the present process negatives of 75 greatly improved quality are obtained. By effecting the re-touching on an image of positive appearance the re-touching, fine etching or re-

ducing operation is greatly facilitated as the positive effect of the photographic image can be seen before the plate is finally printed.

Prepared photo plates produced by the present process can be used for original drawings, sketches, etchings and the like so as to obtain reproductions of very high quality. The finished negatives obtained by the present process may be printed from for use with bichromated glue, 10 albumen, or gum, or silver or other sensitive surfaces.

By use of the methods according to the present invention there can be obtained negatives which in their finished condition are of greater opacity than those produced by the methods heretofore usually employed with dry plates. Further there may be obtained by the present process stencil-like negatives of better quality, especially for use in photo-lithographic work, than those heretofore produced; these stencil-like negatives produced by the present methods give machine plates of more durability than those made from fringed dot negatives which have been retouched with dye or by other methods heretofore usually employed.

It is to be understood that the process according to the present invention is applicable not only to plates but equally to films or paper or other base materials coated with a dried photographic emulsion, and that in the appended claims the term "plate" is used to denote any of the usual base materials (including glass plates, films or paper) coated with a dried photographic emulsion as just mentioned.

What I claim and desire to secure by Letters 35 Patent of the United States is:—

1. A process of treating a negative so as to obtain a photographic image thereon having improved tone-printing values, especially for use in photo-mechanical printing work; which process consists in subjecting a fixed negative to the action of a first solution comprising a bleaching reagent which produces on the plate a silver halide photographic image of positive appearance, then treating the plate with a second solution that is a solvent for the silver halide so as to effect 10 the requisite retouching on the positive image without re-converting it to a negative image, and finally subjecting the plate to the action of a third solution which blackens the silver halide image thereby reconverting the image of positive 15 appearance to a negative image.

2. A process of treating a negative to obtain a photographic image thereon having improved tone printing values, especially for use in photo-mechanical printing work, which consists in first 20 subjecting the negative to the action of a first solution comprising a bleaching reagent which produces on the plate a silver halide photographic image of positive appearance, second, applying a protective coating to those parts of the image 25 which already have the required tone, third, treating the plate with a solution of a solvent for the silver halide image to effect the requisite re-touching on the positive image without reconverting it to a negative image, fourth, removing 30 said coating and fifth, finally subjecting the plate to the action of a solution which blackens the silver halide image thereby reconverting the image of positive appearance to a negative image.

ARTHUR ERNEST FIELD. 35